

Nov. 12, 1957

L. STEVENS

2,812,782

MONOFILAMENT AND FABRIC MADE THEREBY

Filed Feb. 10, 1955

FIG. 1



FIG. 2



FIG. 3



FIG. 4



INVENTOR.  
LESLIE STEVENS

BY *Chapin & Deal*  
ATTORNEYS

# United States Patent Office

2,812,782

Patented Nov. 12, 1957

1

2,812,782

## MONOFILAMENT AND FABRIC MADE THEREBY

Leslie Stevens, Nelson, Lanes, England, assignor to Chicopee Manufacturing Corporation, New Brunswick, N. J., a corporation of Massachusetts

Application February 10, 1955, Serial No. 487,389

Claims priority, application Great Britain  
January 29, 1955

7 Claims. (Cl. 139—420)

This invention relates to a novel filament of synthetic material and to a fabric woven partially or wholly of the same. The fabric of this invention may be used in many ways. Some of the particular uses to which it may be put to advantage are: as an upholstery cloth, such as has been used extensively for automobile seat covering material and the like; as lining fabrics or shirting material in the wearing apparel field; as fabrics for shoes, millinery, handbags, etc.; as a utility cloth for pipe coverings and other wrapping and lining purposes; and as material for window shades, lamp shades and other general decorative trim purposes. This listing is not intended to be all-inclusive, but rather to indicate the wide variety of applications for which the fabric may be adapted both from a decorative as well as a utilitarian standpoint.

An object of the invention is to provide a new type of fabric forming filament for weaving fabrics and specifically a monofilament, flat or elliptical in cross section, of synthetic material, and characterized by a novel formation of kinks disposed at random along the length of the monofilament and imparted thereto by a series of irregularly angled twisted portions.

A further object is to provide an improved fabric for the above and other purposes having an attractive, somewhat pebbly or nubby surface formed by a haphazard spacing of kinks in the filaments and an irregularly disposed angular relationship of adjacent portions of the filament. The filaments may serve either as the warp or weft or both, and fabrics made according to the invention sometimes having a general appearance suggestive of a boucle type of woven fabric.

The above and other specific objects and advantages of the invention will be apparent from the following description thereof in connection with the accompanying drawings, in which,

Fig. 1 is a perspective view on an enlarged scale of a small swatch of the new fabric with the weft filaments made according to this invention;

Fig. 2 is a similar fragmentary view of the new fabric having both warp and weft filaments formed according to the invention;

Fig. 3 is an enlarged view of a short length of a new monofilament showing the disposition of the kinks and nature of the twists formed therein; and

Fig. 4 is a more or less diagrammatic view to illustrate the manner in which kinking may be imparted to a monofilament.

Broadly speaking the present invention resides in the formation of a unique monofilament of synthetic material having a flat or elliptical cross sectional shape and characterized by a series of haphazardly angled and irregularly spaced twisted portions formed therein to impart random localized kinks in the filament. When woven into a fabric the kinks of the filaments give a nubby appearance and feel to the fabric.

In the drawings a single monofilament 1 is shown by Fig. 3. This filament, as indicated, is uniformly flat

2

in cross section throughout its length. It is initially made up in the flattened form according to conventional practices from a synthetic thermoplastic resin material. The plastic materials from which the filament may be made are well known. They are waterproof and chemically resistant, tough and flexible, and are commercially available in filament form. One such material, for example, is available under the trade name "Saran," referring to the copolymer of vinyl chloride and vinylidene chloride. Other plastic materials having similar properties may also be used.

It may be noted from Fig. 3 that the new monofilament is twisted to form a localized kinking at irregularly spaced points along its length. As shown, the portion indicated at 2 is turned with respect to the portion at 3, and the portion at 4 is turned with relation to both portions 3 and 5 respectively. Each portion may be unequal in length with respect to each of its next adjacent portions and furthermore the angular relationship is of a non-uniform character as will appear in comparing portions 2 and 4 with portion 3. The various portions, as described, have been crowded into the illustration of Fig. 3 to emphasize the irregular and random nature of the twisting and kinking in a single filament. It will be understood the various portions enumerated may be of a greater length than those shown. In other words the filaments 1, as will be realized from an inspection of Fig. 1, may be twisted only once or twice along a length of filament equal to that of Fig. 3.

The twisting may be imparted to the filament in a number of ways. One such way is to draw the flat filament "over end" from a form on which it has been wound in the regular way, as for example, on a bobbin, spool or similar package. The filament is thus withdrawn in a direction generally parallel to the axis of the winding, that is laterally and substantially at right angles to the direction of the winding. Thus when a length of filament equal to the circumference of the wound filament is withdrawn, the filament is twisted one complete turn. The twisting action during this type of withdrawing operation kinks the filament and results in a permanently twisted pair of adjacent portions. By a "permanent" twist in the filament, as the term is used herein, is meant a condition under which the structure of the filament is deformed to the extent that the twist therein will be self-sustaining and remain in the filament in the absence of any positive application of forces intended to reverse the twist and erase the kink.

The diagrammatic showing of Fig. 4 with a spool form 6 and a withdrawn portion of filament 1 directed "over end" through an eye 7 is for purposes of illustration. It will be readily appreciated that any known mechanism for twisting filaments may be used such as the conventional twisters of the textile art.

In the twisting of the monofilament 1 the flattened cross sectional shape thereof appears to be a principal factor in obtaining a well defined permanent kink with the portions adjacent thereto being angularly related. In twisting monofilaments of circular cross section the twisting forces are distributed essentially uniformly along the length of the thread. No observable twists or kinks are imparted to a circular filament, nor can any deformation of the material be detected by feeling the same. When used in a fabric no observable decorative effect is achieved by twisted circular filaments. However, with the flattened cross sectional shape, as will be evident from Fig. 3, the kinks and twisted portions can obviously be seen and can definitely be felt between the fingers. A unique decorative effect is thus obtainable in the fabric, see Fig. 1. By the simple method of obtaining a twist as described, the kinks are irregularly located with the angular rela-

tionship between adjacent portions appearing to be either at 90°, at 180° or somewhere between those two limits. Where the angular relationship is at 90° or slightly greater, the surface of the fabric (especially when the monofilaments are used as the filling, see Fig. 1) will be slightly "ridged" to give a rough feel to the woven material and a different contrasting appearance in the area where the warp filaments embrace the edges of the monofilament rather than the flat sides. At each turning or twist of the filament, whether the twist be of 180° or less, there is formed in the immediate area an upraised nub on the surface suggestive of the feel and appearance of a knotted yarn such as is found in the conventional boucle type of material. With the plane of the surface of each monofilament angularly shifting at angles varying from 90° to 180° at various points along its length it will at once be apparent a great variety of different visual effects may be achieved by the number of twists given to each filament and the arrangement of monofilaments in the finished fabric material.

As mentioned, Fig. 1 shows a fabric in which the new monofilaments 1 have been used as the filling. Fig. 2 illustrates the use of filaments 1 in both warp and weft. In Fig. 1 the warp comprises continuous filament viscose rayon threads as at 10. The nature and variety of possible combinations are thus practically without limit.

In weaving the fabric, as will also be appreciated by those skilled in the weaving art, an additional twist may be imparted to a monofilament by shuttle movement and the withdrawal of the filament from a suitable quill. An "over end" withdrawal from a quill imparts a twist after the manner of the twisting illustrated by Fig. 4. Thus when used as filling the additional twist of the flat filament in the weaving operation may be taken into account in forming a particular fabric and planning the number of preliminary withdrawing operations necessary to obtain the desired kinked character of the filament. According to the present invention a wide variety of novel, ornamental, and esthetic effects may thus be achieved.

What is claimed is:

1. As a new article of manufacture a monofilament having a flattened cross sectional shape and disposed along its length a plurality of irregularly spaced twisted kinks, the kinks being localized at random with twisted areas of successive kinks being of varying angularity and the portions between adjacent kinks lying in varying planes.

2. As a new article of manufacture a monofilament having a flattened cross sectional shape with a plurality of irregularly spaced kinks disposed at random along its length, said kinks being formed by localized helically twisted sections of the monofilament with flat portions

therebetween, the twisted portions of the successive kinks being of varying angularity and the successive flat portions lying in varying planes.

3. As a new article of manufacture a monofilament comprising the copolymer of vinyl chloride and vinylidene chloride and having a flattened cross sectional shape with a succession of haphazardly angled twisted sections forming kinked portions at irregularly spaced intervals longitudinally of the length thereof, the portions between said kinked portions being of greater length than the said twisted sections and lying in varying planes.

4. A woven fabric having thermoplastic fabric forming monofilaments of a flattened cross sectional shape with a plurality of kinks twisted at random along the length of the monofilament, the kinks being localized haphazardly with oppositely twisted areas of the successive kinks being of varying angularity and the portions between said twisted areas lying in varying planes.

5. A fabric of warp and weft filaments with the filaments forming one of said types being of synthetic thermoplastic material and in the form of monofilaments characterized by a flattened cross sectional shape with a plurality of irregularly disposed kinks having twisted portions of varying angular relationships along the length thereof with flat portions between said twisted portions of the successive kinks lying in varying planes and imparting nubby surface characteristics to the feel and appearance of said fabric.

6. A woven fabric simulating the nubby surface characteristics of a boucle type woven fabric and having at least the weft thereof comprising thermoplastic filaments, flattened in cross section, and helically twisted haphazardly at random locations along the length thereof with flat portions therebetween, the successive twisted portions being of varying angularity and of less length than the flat portions and the successive flat portions lying in varying planes.

7. A woven fabric comprising a warp having continuous filament viscose rayon threads and a weft having thermoplastic monofilaments formed of the copolymer of vinyl chloride and vinylidene chloride, said monofilaments being of flat cross sectional shape with a plurality of twisted areas kinking the monofilaments at irregularly and randomly spaced positions along the length thereof, said twisted areas being localized haphazardly with the sections of successive areas being of varying angularity and the portions between adjacent twisted areas lying in varying planes.

References Cited in the file of this patent

UNITED STATES PATENTS

2,002,153 Mendel \_\_\_\_\_ May 21, 1935